

## UNITED STATES PATENT OFFICE

2,455,170

## COLORED COUPLERS

Dudley B. Glass, Paul W. Vittum, and Arnold Weissberger, Rochester, N. Y., assignors to Eastman Kodak Company, Rochester, N. Y., a corporation of New Jersey

No Drawing. Application May 3, 1944,  
Serial No. 533,932

7 Claims. (Cl. 95—6)

1

This invention relates to color photography and particularly to coupler compounds for use in photographic processes.

Color-forming compounds which react with the development product of aromatic amino developing agents to form colored images upon photographic development are well known. Generally, these color-forming compounds or couplers are colorless or substantially colorless. This lack of color is usually desirable where the coupler is to be incorporated in the emulsion layer and the unused coupler remains after formation of the colored image. When the coupler is used in the developing solution, it may be colored without detriment to the final image, and some colored couplers are known, such as paraphenylazo acetanilide which was disclosed in Mannes and Godowsky Patent 2,108,602.

We have now found a new type of coupler which may have applications in several fields. The new couplers are, in themselves, more or less strongly colored, and during the coupling reaction, the chromophore system in the coupler is broken up with the result that the original color of the coupler is destroyed and a new dye is formed. Thus, on developing an emulsion layer containing one of these colored couplers, the coupler color is destroyed, and a new color is formed by the coupling reaction, at those points where development occurs. There is formed in this way a dye image of one color on a background of another color.

It is, therefore, an object of the present invention to provide a colored coupler whose chromophore system is destroyed on coupling. A further object is to provide a novel radical replacement type of chemical reaction. A still further object is to provide color couplers suitable for color correction processes of color photography. Other objects will appear from the following description of our invention.

These objects are accomplished by using as the coupler a compound having a heterocyclic system containing a methylene group and an adjacent carbonyl group as part of the ring structure, the methylene group having been substituted with an azo group. These compounds have the following general formula:



where Z represents the atoms necessary to complete a cyclic structure having adjacent the methylene group —S—, —NH—, or a doubly bound carbon atom and R represents an aromatic or heterocyclic radical.

2

More specifically, the compounds which we contemplate using have the following structure:



where X represents the atoms necessary to complete the five-membered ring having adjacent the methylene group —S—, —NH—, or a doubly bound carbon atom and R is the same as before.

In previous descriptions of reactive methylene compounds for color photography, it has been assumed that the reactive methylene group must be unsubstituted in order for coupling with the developer to occur. We have found that the active methylene group may be substituted with an azo group and that this group is removable by the oxidized photographic developer when the azo-substituted coupler is treated with the oxidized developer either in aqueous solution or in the photographic emulsion layer. Thus, the coupler may be converted to a colored compound and the azo group readily removed from it by means of reaction with the oxidized developing agent. This reaction appears to proceed as follows:



where Z and R are the same as in the general formula above.

The following examples illustrate compounds which contain azo-substituted methylene groups according to the general formula above and which may be used to produce colored images according to our invention:

1. 

1-phenyl-3-methyl-4-(X-phenyl-azo)-5-pyrazolone  
X=H, OH, SO<sub>3</sub>H, SO<sub>2</sub>NH<sub>2</sub>, N(CH<sub>3</sub>)<sub>2</sub>, NHCOCH<sub>3</sub>, NO<sub>2</sub>, COOH
2. 

2-phenylazo-1,3-indandione

3.   
1-(p-nitrophenylazo)-2(1)-thionaphthene-1,4-dione
4.   
2-ethyl-4-phenylazo-tetrahydro-1,3-diketoisoquinoline
5.   
2-phenylazo-2,3-dihydro-3-ketoindole (2-phenylazopseudoindoxyl)
6.   
1-ethyl-3-phenylazo-2,3-dihydro-2-ketoindole (1-ethyl-3-phenylazoxindole)
7.   
1-phenyl-3-benzamido-4-(p-amoxypheylazo)-5-pyrazolone
8.   
1-p-(p'-tert-butylphenoxy)-phenyl-3-methyl-4-p-hydroxyphenylazo-5-pyrazolone

Our compounds are intended for incorporation in silver halide emulsion layers either in single layer or multi-layer coatings. The compounds may be added directly to the emulsion as the sodium or other water-soluble salt or they may be incorporated in a coupler solvent as described in Mannes and Godowsky U. S. Patent 2,304,940 or Jelley and Vittum U. S. Patent 2,322,027.

The compounds employed according to our invention may be produced by any suitable method such as by reaction of the reactive methylene compound with the appropriate diazonium compound. For example, compound No. 8 was prepared as follows:

p-Hydroxyaniline (5.5 g.; 0.05 mole) was dissolved in a solution of 40 cc. of water and 15 cc. of concentrated hydrochloric acid and diazotized at 0° C. by the addition of 3.5 g. (0.05 mole) of sodium nitrite. This solution was added to a solution of 16.1 g. (0.05 mole) of 1-(p-(p-tert-butylphenoxy)-phenyl)-3-methyl-5-pyrazolone in 200 cc. of water which contained 10 g. of sodium hydroxide. The temperature of the reaction mixture was kept at 0° C. by the addition of ice. After standing for thirty minutes the cold solution was acidified with 20 cc. of concentrated hydrochloric acid. After the product had crystallized, it was washed with water and dried in air. The yield amounted to 19 g. (86%). The product was recrystallized from acetic acid. M. P. 185-187°.

Our compounds are particularly useful in a process, such as that of Hanson U. S. Patent 2,449,966, granted September 21, 1948. The Hanson process involves a color correction method in which a colored coupler is incorporated in the

photographic emulsion layer prior to exposure and upon development is converted into a colored image where the layer was exposed. The coupler remaining in the unexposed portions of the layer retains its original color; and by suitable choice of the color of the original coupler and the color of the final dye image a masking or correction effect can be obtained.

Various photographic developing agents can be employed with the couplers of our invention. The primary aromatic amino developing agents are generally suitable including the phenylene-diamines and the aminophenols. The alkyl phenylenediamines may be substituted in the amino group as well as in the ring. Suitable compounds are diethyl paraphenylenediamine, monomethyl paraphenylenediamine, dimethyl paraphenylenediamine and para-aminophenol. These compounds are usually employed in the salt form, such as the hydrochloride or the sulphate which are more stable than the free amines. All of these compounds have a primary amino group which enables the oxidation product of the developer to couple with the color-forming compounds to form dye images.

The following developing solution is suitable for developing gelatino silver halide layers containing colored couplers according to our invention.

2-amino-5-diethyl-amino toluene HCl \_\_\_\_\_ grams \_\_\_\_\_ 2  
Sodium sulphite \_\_\_\_\_ do \_\_\_\_\_ 2  
Sodium carbonate \_\_\_\_\_ do \_\_\_\_\_ 20  
Potassium bromide \_\_\_\_\_ do \_\_\_\_\_ 2  
Water to \_\_\_\_\_ liter \_\_\_\_\_ 1

It will be understood that the examples and modifications set forth herein are illustrative only and that our invention is to be taken as limited only by the scope of the appended claims.

We claim:

1. The method of developing a colored image in a silver halide emulsion layer which comprises incorporating in said layer a coupler compound having the formula:



where R is an aryl group, R' is an aryl group of the benzene series and X is an acyl group, and said coupler compound contains no other reactive CH group, exposing said layer and developing it with a primary, aromatic amino developing agent, thereby splitting off the  $\text{N}=\text{N}-\text{R}'$  group in said coupler compound and coupling said coupler compound at the point of splitting with the oxidation product of the primary, aromatic amino developing agent to form a dye image, leaving said coupler compound intact in the undeveloped regions of said layer.

2. The method of developing a colored image in a silver halide emulsion layer which comprises incorporating in said layer a coupler compound having the formula:



where R' is an aryl group of the benzene series and X' is an aromatic acid acyl group, and said coupler compound contains no other reactive CH group, exposing said layer and developing it with a primary aromatic amino developing agent, thereby splitting off the  $\text{N}=\text{N}-\text{R}'$  group in

said coupler compound and coupling said coupler compound at the point of splitting with the oxidation product of the primary aromatic amino developing agent to form a dye image, leaving said coupler compound intact in the undeveloped regions of said layer.

3. The method of developing a masked magenta color separation image in a multilayer photographic element having three superposed silver halide emulsion layers, which comprises incorporating in one of said emulsion layers a coupler compound having the formula:



where Z represents the atoms necessary to complete a cyclic structure in which there is adjacent the reactive CH group a member selected from the class consisting of —S—, —NH—, and carbon doubly bound to an atom selected from the class consisting of (1) a carbon atom which is part of a conjugated chain linked to an electro-negative atom, (2) nitrogen and (3) oxygen, and R is selected from the class consisting of aromatic and heterocyclic radicals, and said coupler compound contains no other reactive CH group, exposing said layer and developing it with a primary aromatic amino developing agent, thereby splitting off the —N=N—R group in said coupler compound and coupling said coupler compound at the point of splitting, with the oxidation product of the primary aromatic amino developing agent to form a magenta dye image, leaving said coupler compound intact in the undeveloped regions of said one layer.

4. The method of developing a masked magenta color separation image in a multilayer photographic element having three superposed silver halide emulsion layers, which comprises incorporating in one of said emulsion layers a coupler compound having the formula:



where X represents the atoms necessary to complete a five-membered ring in which there is adjacent the reactive CH group a member selected from the class consisting of —S—, —NH—, and carbon doubly bound to an atom selected from the class consisting of (1) a carbon atom which is part of a conjugated chain linked to an electro-negative atom, (2) nitrogen and (3) oxygen, and R is selected from the class consisting of aromatic and heterocyclic radicals, and said coupler compound contains no other reactive CH group, exposing said layer and developing it with a primary aromatic amino developing agent, thereby splitting off the —N=N—R group in said coupler compound and coupling said coupler compound at the point of splitting, with the oxidation product of the primary aromatic amino developing agent to form a magenta dye image, leaving said coupler compound intact in the undeveloped regions of said one layer.

5. The method of developing a masked magenta color separation image in a multilayer photographic element having three superposed silver halide emulsion layers, which comprises incorporating in one of said emulsion layers a coupler compound having the formula:



where X represents the atoms necessary to complete a pyrazolone ring, and R is selected from the class consisting of aromatic and heterocyclic radicals, and said coupler compound contains no other reactive CH group, exposing said layer and developing it with a primary aromatic amino developing agent, thereby splitting off the —N=N—R group in said coupler compound and coupling said coupler compound at the point of splitting, with the oxidation product of the primary aromatic amino developing agent to form a magenta dye image, leaving said coupler compound intact in the undeveloped regions of said one layer.

10 6. The method of developing a masked magenta color separation image in a multilayer photographic element having three superposed silver halide emulsion layers, which comprises incorporating in one of said emulsion layers a coupler compound having the formula:



25 25 where R' and R'' are mononuclear aryl groups and Y is selected from the class consisting of methyl and acylamino groups and said coupler compound contains no other reactive CH group, exposing said layer and developing it with a primary aromatic amino developing agent, thereby splitting off the —N=N—R' group in said coupler compound and coupling said coupler compound at the point of splitting, with the oxidation product of the primary aromatic amino developing agent to form a magenta dye image, leaving said coupler compound intact in the undeveloped regions of said one layer.

30 40 7. The method of improving the color rendition of multilayer photographic materials having silver halide emulsion layers in which subtractively colored images are formed, which comprises incorporating in one of said layers a coupler compound having the formula:



45 50 where R represents a mononuclear aryl radical and R'' represents a mononuclear aryl radical, exposing said material and developing it with a developer containing a primary aromatic amino developing agent.

DUDLEY B. GLASS.

PAUL W. VITTM.

ARNOLD WEISSBERGER.

#### REFERENCES CITED

60 The following references are of record in the file of this patent:

#### UNITED STATES PATENTS

| Number    | Name            | Date           |
|-----------|-----------------|----------------|
| 2,213,986 | Kendall et al.  | Sept. 10, 1940 |
| 2,220,123 | Schwarz         | Nov. 5, 1940   |
| 2,262,055 | Sease           | Nov. 11, 1941  |
| 2,271,230 | Petersen et al. | Jan. 27, 1942  |
| 2,308,023 | Peterson        | Jan. 12, 1943  |
| 2,310,943 | Dorough         | Feb. 16, 1943  |
| 2,334,495 | Kendall         | Nov. 16, 1943  |
| 2,369,489 | Porter          | Feb. 13 1945   |

#### OTHER REFERENCES

Ser. No. 394,290, Bruylants et al. (A. P. C.) published May 4, 1943.